



US009519237B2

(12) **United States Patent**  
**Okada**

(10) **Patent No.:** **US 9,519,237 B2**  
(45) **Date of Patent:** **Dec. 13, 2016**

(54) **ELECTROSTATIC LATENT IMAGE DEVELOPING TONER, METHOD FOR MANUFACTURING ELECTROSTATIC LATENT IMAGE DEVELOPING TONER, AND METHOD FOR FIXING ELECTROSTATIC LATENT IMAGE DEVELOPING TONER**

(71) **Applicant:** **KYOCERA Document Solutions Inc.**,  
Osaka (JP)

(72) **Inventor:** **Seiji Okada**, Osaka (JP)

(73) **Assignee:** **KYOCERA Document Solutions Inc.**,  
Osaka (JP)

(\*) **Notice:** Subject to any disclaimer, the term of this patent is extended or adjusted under 35 U.S.C. 154(b) by 169 days.

(21) **Appl. No.:** **14/482,209**

(22) **Filed:** **Sep. 10, 2014**

(65) **Prior Publication Data**

US 2015/0072281 A1 Mar. 12, 2015

(30) **Foreign Application Priority Data**

Sep. 11, 2013 (JP) ..... 2013-188634

(51) **Int. Cl.**

**G03G 9/08** (2006.01)  
**G03G 9/093** (2006.01)  
**G03G 9/097** (2006.01)

(52) **U.S. Cl.**

CPC ..... **G03G 9/09392** (2013.01); **G03G 9/09314** (2013.01); **G03G 9/09328** (2013.01); **G03G 9/09342** (2013.01); **G03G 9/09371** (2013.01); **G03G 9/09708** (2013.01)

(58) **Field of Classification Search**

CPC ..... G03G 9/00804; G03G 9/0804  
See application file for complete search history.

(56) **References Cited**

**U.S. PATENT DOCUMENTS**

5,800,957 A \* 9/1998 Agata ..... G03G 9/09335  
430/108.24  
2005/0271964 A1 12/2005 Etou et al.

**FOREIGN PATENT DOCUMENTS**

|    |               |         |
|----|---------------|---------|
| JP | H02-003077 A  | 1/1990  |
| JP | 2002-091060 A | 3/2002  |
| JP | 2004-294467 A | 10/2004 |
| JP | 2004-294468 A | 10/2004 |
| JP | 2010-181439 A | 8/2010  |
| JP | 2010-191272 A | 9/2010  |
| JP | 2010-262111 A | 11/2010 |

**OTHER PUBLICATIONS**

An Office Action; "Notice of Reasons for Rejection," issued by the Japanese Patent Office on Dec. 8, 2015, which corresponds to Japanese Patent Application No. 2013-188634 and is related to U.S. Appl. No. 14/482,209.

(Continued)

*Primary Examiner* — Hoa V Le

(74) **Attorney, Agent, or Firm:** Studebaker & Brackett  
PC

(57) **ABSTRACT**

An electrostatic latent image developing toner includes toner particles. Each toner particle includes a toner core containing a binder resin, a shell layer coating a surface of the toner core, and needle-like inorganic particulates. Each shell layer contains a thermosetting resin, and the inorganic particulates are present within the shell layer. The inorganic particulates have: an aspect ratio of 1.25 or more and 2.5 or less; and an average major diameter and an average minor diameter of 300 nm or less.

**10 Claims, 5 Drawing Sheets**



(56)

**References Cited**

OTHER PUBLICATIONS

An Office Action; "Notice of Reasons for Rejection," issued by the Japanese Patent Office on Mar. 15, 2016, which corresponds to Japanese Patent Application No. 2013-188634 and is related to U.S. Appl. No. 14/482,209.

\* cited by examiner



FIG. 1



FIG. 2



FIG. 3



FIG. 4



FIG. 5



FIG. 6

## 1

**ELECTROSTATIC LATENT IMAGE  
DEVELOPING TONER, METHOD FOR  
MANUFACTURING ELECTROSTATIC  
LATENT IMAGE DEVELOPING TONER,  
AND METHOD FOR FIXING  
ELECTROSTATIC LATENT IMAGE  
DEVELOPING TONER**

INCORPORATION BY REFERENCE

The present application claims priority under 35 U.S.C. §119 to Japanese Patent Application No. 2013-188634, filed Sep. 11, 2013. The contents of this application are incorporated herein by reference in their entirety.

BACKGROUND

The present disclosure relates to an electrostatic latent image developing toner, a method for manufacturing an electrostatic latent image developing toner, and a method for fixing an electrostatic latent image developing toner.

In the technical field of image forming as in copiers, an electrostatic latent image developing toner is fixed to a recording medium (for example, paper) by applying heat and pressure through a fixing roller, for example. By the heat and pressure applied, the components of the toner melt or soften to be fixed to the recording medium. Desirably, the fixing is done in an energy saving manner and with a smaller fixing device. For this purpose, a toner is desired to be duly fixed to a recording medium while the heat and pressure applied to the fixing roller is kept to a minimum.

As a toner usable for such image forming, a study is underway for a toner including particles each having a surface coated with a urea resin.

In addition, a study is under way for a toner including toner cores each having a surface to which inorganic particulate are externally attached and which is coated with a silane compound.

SUMMARY

The gist of the present disclosure is as follows.

An electrostatic latent image developing toner according to the present disclosure includes toner particles. Each toner particle includes a toner core containing a binder resin, a shell layer coating a surface of the toner core, and needle-like inorganic particulates. Each shell layer contains a thermosetting resin, and the inorganic particulates are present within the shell layer. The inorganic particulates have: an aspect ratio of 1.25 or more and 2.5 or less; and an average major diameter and an average minor diameter of 300 nm or less.

According to the present disclosure, a method for manufacturing an electrostatic latent image developing toner involves: preparing toner cores containing a binder resin; and forming shell layers to coat surfaces of the respective toner cores. The shell layers contain a thermosetting resin, and needle-like inorganic particulates are present within the shell layers. The inorganic particulates have an aspect ratio of 1.25 or more and 2.5 or less and an average major diameter and an average minor diameter of 300 nm or less.

According to the present disclosure, a method for fixing an electrostatic latent image developing toner to a recording medium involves: supplying the electrostatic latent image developing toner to a surface of a recording medium; and applying a load of 5 N/cm<sup>2</sup> or more and 10 N/cm<sup>2</sup> or less to

## 2

the recording medium to which the electrostatic latent image developing toner has been supplied.

BRIEF DESCRIPTION OF THE DRAWINGS

5

FIG. 1 shows a toner particle of an electrostatic latent image developing toner according to an embodiment.

FIG. 2 illustrates a method for measuring a softening point by using an elevated flow tester.

10

FIG. 3 shows a toner particle of an electrostatic latent image developing toner according to another embodiment.

FIG. 4 is a schematic view of a fixing unit used in a fixing method according to an embodiment.

15

FIG. 5 is a scanning electron microscope (SEM) photograph of an electrostatic latent image developing toner prepared in Example 1.

20

FIG. 6 is an SEM photograph of a surface of a toner particle contained in the electrostatic latent image developing toner prepared in Example 1 and then fixed to a recording medium.

DETAILED DESCRIPTION

The following describes embodiments of the present disclosure in detail. The present disclosure is not limited to the embodiments described below, and various alterations may be appropriately made without departing from the object of the present disclosure. Note that some overlapping explanations may be appropriately omitted, but such omission is not intended to limit the gist of the disclosure.

An electrostatic latent image developing toner (which hereinafter may be referred to simply as "toner") according to an embodiment includes toner particles. Each toner particle includes a toner core containing a binder resin, a shell layer coating a surface of the toner core, and needle-like inorganic particulates. Each shell layer contains a thermosetting resin, and the inorganic particulates are present within the shell layer. The needle-like inorganic particulates have an aspect ratio of 1.25 or more and 2.5 or less and also have an average major diameter and an average minor diameter of 300 nm or less. According to the present embodiment, the toner cores are anionic (negatively chargeable), whereas the shell layers are cationic (positively chargeable).

45 The following describes the electrostatic latent image developing toner according to the present embodiment, with reference to FIG. 1.

The electrostatic latent image developing toner includes toner particles 1. As shown in FIG. 1, each toner particle 1 contains a toner core 2, a shell layer 3, and inorganic particulates 4. The shell layer 3 contains a thermosetting resin and coats the surface of the toner core 2. Each inorganic particulate 4 has a needle-like shape.

With the presence of the shell layer 3 containing a thermosetting resin having a high hardness, the toner particle 1 exhibits excellent blocking resistance, conveyance, preservability, and so on. The electrostatic latent image developing toner according to the present embodiment is supplied to a recording medium, such as paper, and the shell layers 3 rupture in response to the application of heat and load. As a result of the rupture of the shell layers 3, the toner cores 2 are exposed and melt or soften, so that the toner is fixed to the recording medium.

Each inorganic particulate 4 in the toner particle 1 may 65 serve as a starting point of the rupture. Therefore, although the shell layer 3 coating the surface of the toner core 2 contains a high hardness thermosetting resin, the shell layer

3 can be easily ruptured. This ensures the toner cores 2 to be sufficiently fixed to a recording medium while the temperature and load necessary for fixing the toner image to the recording medium are significantly reduced. In addition, owing to its needle-like shape, the inorganic particulates 4 compare favorably with spherical inorganic particulates in the function of releasing excessive charges. Therefore, the toner according to the present embodiment can maintain appropriate chargeability for a long time.

The following describes the toner core 2.

The toner cores 2 contain a binder resin as an essential component. The binder resin is anionic. The binder resin has a functional group which, for example, is an ester group, a hydroxyl group, a carboxyl group, an amino group, an ether group, an acid group, or a methyl group. The binder resin preferably has a functional group, such as a hydroxyl group, a carboxyl group or an amino group, in a molecule, and more preferably has a hydroxyl group and/or a carboxyl group in a molecule. Such a function group is favorable because it reacts with a unit derived from a monomer of the thermo-setting resin (for example, methylol melamine) contained in the shell layer 3 to be chemically bounded. As a result, the shell layer 3 and the toner core 2 of each toner particle 1 are strongly bonded to each other.

When the binder resin has a carboxyl group, for the toner core 2 to be sufficiently anionic, the acid value of the binder resin is preferably 3 mgKOH/g or more and 50 mgKOH/g or less, and more preferably 10 mgKOH/g or more and 40 mgKOH/g or less.

When the binder resin has a hydroxyl group, for the toner cores 2 to be sufficiently anionic, the hydroxyl value of the binder resin is preferably 10 mgKOH/g or more and 70 mgKOH/g or less, and more preferably 15 mgKOH/g or more and 50 mgKOH/g or less.

Specific examples of the binder resin include thermoplastic resins (styrene-based resins, acrylic-based resins, styrene acrylic-based resins, polyethylene-based resins, polypropylene-based resins, vinyl chloride-based resins, polyester resins, polyamide-based resins, polyurethane-based resins, polyvinyl alcohol-based resins, vinyl ether-based resins, N-vinyl-based resins, and styrene-butadiene-based resins). As the binder resin, styrene acrylic-based resins and/or polyester resins are preferred for improving the dispersibility of a colorant in the toner, the chargeability of the toner, and the fixability of the toner to a recording medium.

A styrene acrylic-based resin is a copolymer of a styrene-based monomer and an acrylic-based monomer. Specific examples of the styrene-based monomer include styrene,  $\alpha$ -methylstyrene, p-hydroxystyrene, m-hydroxystyrene, vinyl toluene,  $\alpha$ -chlorostyrene, o-chlorostyrene, m-chlorostyrene, p-chlorostyrene, and p-ethylstyrene.

Specific examples of the acrylic-based monomer include (meth)acrylic acid; (meth)acrylic acid alkyl ester (such as methyl (meth)acrylate, ethyl (meth)acrylate, n-propyl (meth)acrylate, iso-propyl (meth)acrylate, n-butyl (meth)acrylate, iso-butyl (meth)acrylate, and 2-ethylhexyl (meth)acrylate); and (meth)acrylic acid hydroxyalkyl ester (such as 2-hydroxyethyl (meth)acrylate, 3-hydroxypropyl (meth)acrylate, 2-hydroxypropyl (meth)acrylate, and 4-hydroxypropyl (meth)acrylate). Note that "(meth)acrylic acid" includes within the scope of its meaning acrylic acid and methacrylic acid and that "(meth)acrylate" includes within the scope of its meaning acrylate and methacrylate.

In preparation of the styrene acrylic-based resin, a hydroxy group can be introduced into the styrene acrylic-based resin by using a monomer having a hydroxyl group (such as p-hydroxystyrene, m-hydroxystyrene, or hydroxy-

alkyl (meth)acrylate). By appropriately adjusting the amount of the monomer having a hydroxyl group, the hydroxyl value of the resultant styrene acrylic-based resin can be adjusted.

5 In preparation of the styrene acrylic-based resin, a carboxyl group can be introduced into the styrene acrylic-based resin by using (meth)acrylic acid as the monomer. By appropriately adjusting the amount of the (meth)acrylic acid to be used, the acid value of the resultant styrene acrylic-based resin can be adjusted.

10 The polyester resin is obtained through condensation polymerization or co-condensation polymerization of a dihydric or trihydric or higher-hydric alcohol component and a dibasic or tribasic or higher-basic carboxylic acid component.

15 Examples of the dihydric alcohol component include diols (ethylene glycol, diethylene glycol, triethylene glycol, 1,2-propanediol, 1,3-propanediol, 1,4-butanediol, neopentyl glycol, 1,4-butenediol, 1,5-pentanediol, 1,6-hexanediol, 1,4-cyclohexanediethanol, dipropanediol, polyethylene glycol, polypropanediol, and polytetramethylene glycol); and bisphenols (bisphenol A, hydrogenated bisphenol A, polyoxyethylene-modified bisphenol A, and polyoxypropylene-modified bisphenol A). Examples of the trihydric or higher-hydric alcohol component include sorbitol, 1,2,3,6-hexanetrol, 1,4-sorbitan, pentaerythritol, dipentaerythritol, tripentaerythritol, 1,2,4-butanetriol, 1,2,5-pantanetriol, glycerol, diglycerol, 2-methylpropanetriol, 2-methyl-1,2,4-butanetriol, trimethylolethane, trimethylolpropane, and 1,3,5-trihydroxymethylbenzene.

20 Examples of the dibasic carboxylic acid component include maleic acid, fumaric acid, citraconic acid, itaconic acid, glutaconic acid, phthalic acid, isophthalic acid, terephthalic acid, cyclohexane dicarboxylic acid, succinic acid, adipic acid, sebacic acid, azelaic acid, malonic acid, and alkyl succinic acid or alkenyl succinic acid (such as n-butyl succinic acid, n-butenyl succinic acid, isobutyl succinic acid, isobutenyl succinic acid, n-octyl succinic acid, n-octenyl succinic acid, n-dodecyl succinic acid, n-dodecyl succinic acid, isododecyl succinic acid, or isododecyl succinic acid). Examples of the tribasic or higher-basic carboxylic acid component include 1,2,4-benzenetricarboxylic acid (trimellitic acid), 1,2,5-benzenetricarboxylic acid, 2,5,7-naphthalenetricarboxylic acid, 1,2,4-naphthalenetricarboxylic acid, 1,2,4-butanetricarboxylic acid, 1,2,5-hexanetricarboxylic acid, 1,3-dicarboxyl-2-methyl-2-methylene carboxy propane, 1,2,4-cyclohexanetricarboxylic acid, tetra(methylenecarboxyl) methane, 1,2,7,8-octanetetra carboxylic acid, pyromellitic acid, and Empol trimer acid. The carboxylic acid components may be used in the form of an ester-forming derivative (such as an acid halide, an acid anhydride, or a lower alkyl ester). The term "lower alkyl" used herein refers to an alkyl group having 1 to 6 carbon atoms.

25 55 The acid value and the hydroxyl value of the polyester resin can be adjusted by appropriately changing the amount of a dihydric or trihydric or higher-hydric alcohol component and a dibasic or tribasic or higher-basic carboxylic acid component to be used to produce the polyester resin. The acid value and the hydroxyl value of the polyester resin tend to be lower by increasing the molecular weight of the polyester resin.

60 When the binder resin is a polyester resin, the number average molecular weight  $M_n$  of the polyester resin is preferably 1,200 or more and 2,000 or less for improving the strength of the toner cores 2 and the fix ability of the toner particles 1. For the same reason, the molecular weight

distribution of the polyester resin (Mw/Mn, which is the ratio of the mass average molecular weight Mw to the number average molecular weight Mn) is preferably 9 or more and 20 or less.

When the binder resin is a styrene acrylic-based resin, the number average molecular weight Mn of the styrene acrylic-based resin is preferably 2,000 or more and 3,000 or less for improving the strength of the toner cores **2** and the fixability of the toner particles **1**. For the same reason, the molecular weight distribution of the styrene acrylic-based resin (Mw/Mn, which is the ratio of the mass average molecular weight Mw to the number average molecular weight Mn) is preferably 10 or more and 20 or less. Note that the number average molecular weight Mn and the mass average molecular weight Mw of the binder resin can be measured by using gel permeation chromatography.

The glass transition point Tg of the binder resin is preferably equal to or lower than the curing start temperature of the thermosetting resin contained in the shell layer **3** for improving the low-temperature fixability. With the binder resin having the glass transition point Tg falling within the above range, the toner exhibits sufficient low-temperature fixability at the time of high-speed fixing. In particular, the glass transition point Tg of the binder resin is preferably 20° C. or more, and more preferably 30° C. or more and 55° C. or less, and further more preferably 30° C. or more and 50° C. or less. When the glass transition point Tg of the binder resin is 20° C. or more, aggregation of the toner cores **2** during the formation of the shell layers **3** are suppressed. Typically, the curing start temperature of a thermosetting resin is on the order of 55° C.

The glass transition point Tg of the binder resin can be determined based on the point of change in the specific heat of the binder resin measured by using a differential scanning calorimeter (DSC). More specifically, a differential scanning calorimeter (for example, "DSC-6200" manufactured by Seiko Instruments Inc.) can be used as the measuring device to measure the heat absorption curve of the binder resin to determine the glass transition point Tg of the binder resin. Alternatively, the glass transition point Tg of the binder resin can be measured in the following manner. First, a 10 mg measurement sample (the binder resin) is put in an aluminum pan. With an empty aluminum pan used as a reference, a heat absorption curve of the binder resin is obtained within a measurement temperature range of 25° C. to 200° C. and a heating rate of 10° C./min. Then, based on the heat absorption curve thus obtained, the glass transition point Tg of the binder resin can be determined.

The softening point Tm of the binder resin is preferably 100° C. or less, and more preferably 95° C. or less. With the binder resin having the softening point Tm of 100° C. or less, the toner exhibits sufficient low-temperature fixability at the time of high-speed fixing. The softening point Tm of the binder resin can be adjusted by, for example, combining a plurality of resins having different softening points Tm.

The softening point Tm of the binder resin can be measured by using an elevated flow tester (for example, "CFT-500D" manufactured by Shimadzu Corporation). More specifically, a measurement sample (binder resin) is set on the elevated flow tester, 1 cm<sup>3</sup> of the sample is melt flown under predetermined conditions (dies diameter: 1 mm, plunger load: 20 kg/cm<sup>2</sup>, and heating rate: 6° C./min) to obtain an S shaped curve (S shaped curve plotted on the temperature (° C.)/stroke (mm)) The softening point Tm of the binder resin is read from the S shaped curve.

With reference to FIG. 2, the following describes how to read the softening point Tm of the binder resin. In FIG. 2, S<sub>1</sub>

represents the maximum value of the stroke, and S<sub>2</sub> represents a stroke value corresponding to a base line at the lower temperature side than the temperature of S<sub>1</sub>. On the S shaped curve, a temperature corresponding to a stroke value given by (S<sub>1</sub>+S<sub>2</sub>)/2 is determined as the softening point Tm of the measurement sample (binder resin).

Still with reference to FIG. 1, the following describes the toner particle **1**.

The toner core **2** may contain, as a colorant, a known pigment or dye corresponding to the color of the electrostatic latent image developing toner. An example of the black colorant includes carbon black. Also, a combination of colorants, such as a later-described yellow colorant, magenta colorant, and cyan colorant adjusted to be black is usable as the black colorant.

When the electrostatic latent image developing toner is a color toner, the colorant contained in the toner cores **2** may be a yellow colorant, a magenta colorant, a cyan colorant, or the like.

Examples of the yellow colorant include condensed azo compounds, isoindolinone compounds, anthraquinone compounds, azo metal complexes, methine compounds, and allylamide compounds. Specific examples include C.I. Pigment Yellow (3, 12, 13, 14, 15, 17, 62, 74, 83, 93, 94, 95, 97, 109, 110, 111, 120, 127, 128, 129, 147, 151, 154, 155, 168, 174, 175, 176, 180, 181, 191, or 194), Naphthol Yellow S, Hansa Yellow U, and C.I. Bat Yellow.

Examples of the magenta colorant include condensed azo compounds, diketopyrrolopyrrole compounds, anthraquinone compounds, quinacridone compounds, basic dye lake compounds, naphthol compounds, benzimidazolone compounds, thioindigo compounds, and perylene compounds. Specific example includes C.I. Pigment Red (2, 3, 5, 6, 7, 19, 23, 48:2, 48:3, 48:4, 57:1 81:1, 122, 144, 146, 150, 166, 169, 177, 184, 185, 202, 206, 220, 221, or 254).

Examples of the cyan colorant include copper phthalocyanine compounds, copper phthalocyanine derivatives, anthraquinone compounds, and basic dye lake compounds. Specific examples include the cyan colorant include C.I. Pigment Blue (1, 7, 15, 15:1, 15:2, 15:3, 15:4, 60, 62, or 66), phthalocyanine blue, C.I. Bat Blue, and C.I. Acid Blue.

The content of the colorant in the toner core **2** is preferably 1 part by mass or more and 10 parts by mass or less with respect to 100 parts by mass of the binder resin, and more preferably 3 parts by mass or more and 7 parts by mass or less.

The toner core **2** may contain a release agent for improving the fixability of the electrostatic latent image developing toner as well as for suppressing occurrence of offset or image smearing (smudge of printed image caused by rubbing). Examples of the release agent include: aliphatic hydrocarbon-based waxes (such as low molecular weight polyethylene, low molecular weight polypropylene, polyolefin copolymers, polyolefin wax, microcrystalline wax, paraffin wax, and Fischer-Tropsch wax); oxides of the aliphatic hydrocarbon-based waxes (such as polyethylene oxide wax, and a block copolymer of polyethylene oxide wax); vegetable waxes (such as candelilla wax, carnauba wax, haze wax, jojoba wax, and rice wax); animal waxes (such as beeswax, lanolin, and spermaceti wax); mineral waxes (such as ozokerite, ceresin, and petrolatum); waxes containing a fatty acid ester as a principal component (such as montanic acid ester wax, and castor wax); and waxes obtained by deoxidizing part or whole of fatty acid ester (such as deoxidized carnauba wax).

When the toner core **2** contains a release agent, the content of the release agent is preferably 1 part by mass or more and 5 parts by mass or less with respect to 100 parts by mass of the binder resin.

The toner core **2** may contain a charge control agent as needed. The presence of the charge control agent improves the charge level or the charge rising property to yield a toner having excellent durability or stability. The charge rising property serves as an index of whether or not the toner can be charged to a predetermined charge level in a short period of time. Since the toner core **2** is anionic (negatively chargeable), a negatively chargeable charge control agent is usable.

The toner core **2** may contain magnetic powder as needed. When the toner cores **2** containing magnetic powder are used to prepare the toner particles **1**, the electrostatic latent image developing toner containing the toner cores **2** is used as a magnetic one-component developer. Suitable examples of the magnetic powder include iron (such as ferrite or magnetite), ferromagnetic metals (such as cobalt or nickel), alloys containing iron and/or a ferromagnetic metal, compounds containing iron and/or a ferromagnetic metal, ferromagnetic alloys having been ferromagnetized by for example heating, and chromium dioxide.

The particle diameter of the magnetic powder is preferably 0.1  $\mu\text{m}$  or more and 1.0  $\mu\text{m}$  or less, and more preferably 0.1  $\mu\text{m}$  or more and 0.5  $\mu\text{m}$  or less. The magnetic powder having a particle diameter falling within the above range is readily and uniformly dispersed in the binder resin.

In an electrostatic latent image developing toner used as a one-component developer, the content of the magnetic powder is preferably 35 parts by mass or more and 60 parts by mass or less with respect to 100 parts by mass of the total amount of the toner, and more preferably 40 parts by mass or more and 60 parts by mass or less. In an electrostatic latent image developing toner used as a two-component developer, the content of the magnetic powder is preferably 20 parts by mass or less with respect to 100 parts by mass of the total amount of the toner, and more preferably 15 parts by mass or less.

The following describes the shell layer **3**.

The shell layer **3** contains a thermosetting resin as an essential component. The thermosetting resin has a sufficient strength and hardness and is cationic. Throughout the specification and the claims of the present application, the thermosetting resin contains a unit obtained by introducing a methylene group ( $-\text{CH}_2-$ ) derived from formaldehyde into a monomer such as melamine, for example.

Examples of the thermosetting resin include a melamine resin, a urea resin (urea resorcinol-based resin), a guanamine resin, a urethane resin, an amide resin, an olefin resin, and a gelatin-gum arabic resin. As the thermosetting, a melamine resin or a urea resin is preferred as such a resin does not require a significant increase in the fixing temperature.

A melamine resin is a polycondensate of melamine and formaldehyde, and one of the monomers used for forming a melamine resin is melamine. A urea resin is a polycondensate of urea and formaldehyde, and one of the monomers used for forming a urea resin is urea. The melamine or urea may be denatured in a known manner.

The shell layer **3** may contain a resin other than the thermosetting resin as needed, on condition that the presence of such a resin does not impair the effect of the present disclosure. The content of the thermosetting resin in the shell layer **3** is preferably 90% by mass or more and 100% by mass or less with respect to the total amount of the shell layer **3**, and more preferably 95% by mass or more and

100% by mass or less. With the thermosetting resin content of 90% by mass or more, the shell layer **3** will have a sufficient hardness.

The presence of nitrogen atoms in a material facilitates the material to be positively charged to a desired level. Therefore, the shell layer **3** preferably contains nitrogen atoms derived from melamine or urea. To positively charge the shell layer **3** to a sufficient level, the content of the nitrogen atoms in the shell layer **3** is preferably 10% by mass or more.

For example, the thickness  $t$  of the shell layer **3** may be 7 nm or more and 80 nm or less. The thickness  $t$  of the shell layer **3** can be measured by, for example, analyzing a cross-sectional TEM image of the toner particle **1** with commercially available image analyzing software (for example, "WinROOF" manufactured by MITANI CORPORATION).

The following describes the inorganic particulates **4**.

First, the shape of the inorganic particulates **4** is described.

The inorganic particulates **4** each have a needle-like shape, and the aspect ratio (average major diameter/average minor diameter) thereof is 1.25 or more and 2.5 or less. Preferably, the aspect ratio of the inorganic particulate **4** is 1.3 or more and 2.0 or less. With the aspect ratio of 1.25 or more, the shape of each inorganic particulate **4** is ensured not to approach spherical, which is effective to avoid reduction of the charge leakage and thus to avoid the accumulation of charges on the electrostatic latent image developing toner. As a result, the amount of charges on the electrostatic latent image developing toner does not excessively increase (the toner is not overcharged), so that image forming can be conducted appropriately. In addition, since the shape of each inorganic particulate **4** is ensured to not to approach spherical, the stress on the inorganic particulate **4** concentrates locally. This facilitates the shell layer **3** to rupture starting from a location where an inorganic particulate **4** is present, which can significantly improve the low-temperature fixability of the electrostatic latent image developing toner.

With the inorganic particulates **4** having an aspect ratio of 2.5 or less, the charge leakage is not excessively promoted. Therefore, the reduction in the amount of charge on the electrostatic latent image developing toner can be suppressed. As a result, the residual amount of the electrostatic latent image developing toner on a developing sleeve is kept small and thus the electrostatic latent image developing toner can be appropriately collected. This is effective to suppress occurrence of ghost in the developing process.

The average major diameter and the average minor diameter of the inorganic particulates **4** are both 300 nm and less, on condition that the above aspect ratio is satisfied. With the average major diameter and the average minor diameter of 300 nm or less, the inorganic particulates **4** are ensured to be less prone to detachment from the shell layer **3** even when, for example, pressure is applied thereto in the developing device. As a result, the charge leakage can be stably maintained at an appropriate level, and thus the appropriate chargeability can be maintained for a long time. In addition, since the detachment of the inorganic particulates **4** from the shell layer **3** is prevented, the toner cores **2** are not exposed. Consequently, the electrostatic latent image developing toner is prevented from adhering to the developing sleeve and protected from degradation in preservability. In addition, such an average major diameter and an average minor diameter ensure that the inorganic particulates **4** are contained intact in the shell layer **3** without sticking out. If the inorganic particulates **4** are detached or broken, the stress

applied to the shell layer **3** is reduced and thus the shell layer **3** may not be ruptured easily. This reduces the low-temperature fixability of the electrostatic latent image developing toner.

In particular, the average major diameter of the inorganic particulates **4** is preferably 50 nm or more and 290 nm or less. With the inorganic particulates **4** having an average major diameter of 50 nm or more, the shell layer **3** can be ruptured easily. With the inorganic particulates **4** having an average major diameter of 290 nm or less, the charge leakage can be stably maintained at an appropriate level, and thus the low-temperature fixability of the electrostatic latent image developing toner can be maintained without reduction. In addition, the average minor diameter of the inorganic particulates **4** is preferably 20 nm or more and 130 nm or less. With the inorganic particulates **4** having an average minor diameter of 20 nm or more, the shell layer **3** can be ruptured easily. With the inorganic particulates **4** having an average minor diameter of 130 nm or less, the charge leakage can be stably maintained at an appropriate level, and thus the low-temperature fixability of the electrostatic latent image developing toner can be maintained without reduction.

The following describes one example of a method for measuring the average major diameter and the average minor diameter of the inorganic particulates **4**. First, 50 particulates are randomly selected from a set of inorganic particulates **4**. Then, the thus selected 50 inorganic particulates **4** are photographed by using a scanning electron microscope (for example, "JSM-880" manufactured by JEOL Ltd.) at  $\times 50,000$  magnification. Then, the major and minor diameters of the inorganic particulates **4** are measured on the magnified photographs by using commercially available image analyzing software (for example, "WinROOF" manufactured by MITANI CORPORATION). The respective averages of the thus measured diameters are determined as the average major diameter and the average minor diameter. In addition, the aspect ratio of the inorganic particulates **4** can be given by dividing the average major diameter by the average minor diameter.

The amount of the inorganic particulates **4** contained in the shell layers **3** is preferably 0.1% by mass or more and 5.0% by mass or less with respect to the total amount of the toner particles **1**, and more preferably 0.1% by mass or more and 4.5% by mass or less. With the shell layers **3** containing the inorganic particulates **4** in an amount of 0.1% by mass or more of the toner particles **1**, the shell layers **3** can be easily ruptured. This allows the temperature and load necessary for fixing to be significantly reduced. On the other hand, with the shell layers **3** containing the inorganic particulates **4** in an amount of 5.0% by mass or less of the toner particles **1**, excessive charge-up of the resultant electrostatic latent image developing toner can be suppressed and the reduction of density of image to be formed can be suppressed.

Preferably, the inorganic particulates **4** have a higher hardness than the shell layer **3**. The sufficient hardness of the inorganic particulates **4** is preferably one grade higher than that of the shell layer **3** as measured according to JIS K5600 (pencil hardness test), and more preferably at least two grades higher.

Examples of the inorganic particulates **4** include particulates of metal oxides (such as alumina, titanium oxide, magnesium oxide, zinc oxide, strontium titanate, and barium titanate) and particulates of an inorganic material, such as silica.

As the inorganic particulates **4**, needle-like particulates of titanium oxide is preferred as such particulates offer great versatility and easy shape control. The following describes an example of a method for preparing needle-like particulates of titanium oxide.

First, metatitanic acid is prepared by using a known method, such as a sulfuric acid method. To the resulting metatitanic acid, an aqueous solution of sodium hydroxide is added, followed by heating. Then, the thus heated metatitanic acid is sufficiently washed with pure water. Then, hydrochloric acid is added to the thus washed metatitanic acid, followed by further heating. The resultant mixture is cooled and neutralized with the aqueous solution of sodium hydroxide until the pH reaches 7, followed by another 10 washing and heating. Through the above, rutile-type titanium oxide is prepared. Next, to the rutile-type titanium oxide, sodium chloride and tetrasodium pyrophosphate decahydrate are added and mixed. The thus resultant mixture is baked and the resultant baked product is put into pure 15 water and heated again. Then, the resultant beaked product is washed with pure water to remove soluble salt. As a result, 20 needle-like particulates of titanium oxide are prepared.

With a higher baking temperature, the resultant needle-like particulates of titanium oxide will have a larger major diameter and a larger minor diameter. With a lower baking temperature, the resultant needle-like particulates of titanium oxide will have a smaller major diameter and a smaller minor diameter.

The number of inorganic particulates **4** contained in a 25 shell layer **3** can be calculated based on the bulk density of the inorganic particulates **4**. The number of inorganic particulates **4** contained in the shell layer **3** is 50,000 or more and 550,000 or less per toner particle, for example.

The shell layer **3** may contain a charge control agent. 30 Since the shell layer **3** is cationic (positively chargeable), a positively chargeable charge control agent can be contained.

FIG. 3 shows a toner particle **5** contained in an electrostatic latent image developing toner according to another embodiment. As shown in FIG. 3, each toner particle **5** 40 contains a toner core **2**, a shell layer **3**, inorganic particulates **4**, and an external additive **6**. More specifically, the surface of the shell layer **3** is treated by externally adding the external additive **6** for improving the fluidity and handleability. The external addition treatment with the external 45 additive **6** is not particularly limited and a known method can be used. More specifically, the external addition treatment is performed by using a mixer (for example, FM mixer or Nauta mixer (registered trademark)) under the conditions ensuring that the external additive **6** is not embedded in the shell layer **3**.

Examples of the external additive **6** include the particles of silica and metal oxides (such as alumina, titanium oxide, magnesium oxide, zinc oxide, strontium titanate, and barium titanate). The particle diameter of the external additive **6** is 55 preferably 0.01  $\mu\text{m}$  or more and 1.0  $\mu\text{m}$  or less.

The toner particle **5** before the treatment with the external additive **6** (a toner particle containing the toner core **2**, the shell layer **3**, and the inorganic particulates **4**) may be referred to as a "toner mother particle". The amount of the external additive **6** to be used is preferably 1 part by mass or more and 10 parts by mass or less with respect to 100 parts by mass of the toner mother particles, and more preferably 2 parts by mass or more and 5 parts by mass or less.

Up to this point, the description is given of the toner particles **1** and the toner particles **5** contained in the electrostatic latent image developing toners according to the present disclosure with reference to FIGS. 1 to 3. Each 60

## 11

electrostatic latent image developing toner according to the present disclosure may further contain magnetic powder, such as ferrite or magnetite, to be used as a one-component developer. Alternatively, each electrostatic latent image developing toner according to the present disclosure may be mixed with a desired carrier to be used as a two-component developer.

As for the carrier, the magnetic carrier is preferred. Specific examples of the magnetic carrier include one containing carrier cores coated with a resin. Examples of the carrier core include: particles of iron, oxidized iron, reduced iron, magnetite, copper, silicon steel, ferrite, nickel, or cobalt; particles of alloys of one or more of these materials and a metal, such as manganese, zinc, or aluminum; particles of iron-nickel alloys or iron-cobalt alloys; particles of ceramics, such as titanium oxide, aluminum oxide, copper oxide, magnesium oxide, lead oxide, zirconium oxide, silicon carbide, magnesium titanate, barium titanate, lithium titanate, lead titanate, lead zirconate, and lithium niobate; and particles of high-dielectric substances, such as ammonium dihydrogen phosphate, potassium dihydrogen phosphate, and Rochelle salt. In addition, a resin carrier containing any of the particles mentioned above (magnetic particles) dispersed in a resin is usable as the material of a carrier core.

Examples of the resin that coats the carrier core include (meth)acrylic-based polymers, styrene-based polymers, styrene-(meth)acrylic-based copolymers, olefin-based polymers (polyethylene, chlorinated polyethylene, and polypropylene), polyvinyl chloride, polyvinyl acetate, polycarbonate, cellulose resins, polyester resins, unsaturated polyester resins, polyamide resins, polyurethane resins, epoxy resins, silicone resins, fluorine resins (polytetrafluoroethylene, polychlorotrifluoroethylene, and polyvinylidene fluoride), phenol resins, xylene resins, diallylphthalate resins, polyacetal resins, and amino resins. These resins may be used singly or two or more types may be used in combination. Note that “(meth)acrylic-based” includes within the scope of its meaning acrylic-based and methacrylic-based. The resin that coats the carrier cores is preferably a silicone resin.

In particular, the amount of the resin that coats the carrier core is preferably 1 part by mass or more and 5 parts by mass or less with respect to 100 parts by mass of the carrier core.

The particle diameter of each carrier measured by using an electron microscope is preferably 20  $\mu\text{m}$  or more and 120  $\mu\text{m}$  or less, and more preferably 25  $\mu\text{m}$  or more and 80  $\mu\text{m}$  or less.

When each electrostatic latent image developing toner according to the present disclosure is used as a two-component developer, the amount of the electrostatic latent image developing toner to be used is preferably 5% by mass or more and 20% by mass or less with respect to the total mass of the two-component developer, and more preferably 5% by mass or more and 12% by mass or less.

Each electrostatic latent image developing toner according to the present disclosure contains toner particles each having a surface coated with a shell layer containing a hard thermosetting resin. Despite that, the toner can be duly fixed at a sufficiently low fixing temperature and a sufficiently small fixing load (pressure applied for fixing), and yet an appropriate chargeability can be maintained for a long time. Each electrostatic latent image developing toner according to the present disclosure can be favorably used in an image forming method, such as an electrophotographic method. In addition, owing to its characteristics, each electrostatic latent image developing toner according to the present disclosure

## 12

is particularly suitable for use in an image forming apparatus having a development section of a touchdown development system.

The touchdown development system refers to the development system as follows. In the touchdown development system, while a two-component developer (a developer containing a toner and a carrier) is carried on a magnetic roller, the toner contained in the two-component developer is transferred alone to a development sleeve to form a thin film of the toner on thereon. Then, the toner forming the thin film is caused to scatter over the surface of a photosensitive drum on which an electrostatic latent image has been formed. As a result, the electrostatic latent image is developed into a toner image. In the touchdown development system, the amount of residual toner on the development sleeve increases with an increase in the amount of charges on the toner. Consequently, the residual toner may not be sufficiently collected from the development sleeve, which tends to end up with occurrence of ghost in the developing process. Yet, with each electrostatic latent image developing toner according to the present disclosure, overcharging of the toner can be suppressed and thus occurrence of ghost in the developing process can be suppressed for a long time, even if the touchdown development system is employed for the development.

With reference to FIG. 1, the following describes a method for manufacturing an electrostatic latent image developing toner, according to the present embodiment.

According to the present embodiment, the method for manufacturing an electrostatic latent image developing toner involves a preparatory process (preparing) and a formation process (forming). In the preparatory process, toner cores **2** containing a binder resin are prepared. In the formation process, shell layers **3** are formed to coat the surfaces of the respective toner cores **2**. In the electrostatic latent image developing toner manufactured by the method according to the present embodiment, the shell layer **3** of each toner particle contains a thermosetting resin, and needle-like inorganic particulates **4** are present within the shell layer **3**. The needle-like inorganic particulates **4** have an aspect ratio of 1.25 or more and 2.5 or less and also have the average major diameter and the average minor diameter of 300 nm or less.

To conduct the preparatory process, it is sufficient that components other than the binder resin (such as a colorant, charge control agent, release agent, and/or magnetic powder) are dispersed well in the binder resin. Examples of the method employed for conducting the preparatory process include a melting and kneading method and a polymerization method.

The melting and kneading method is employed in the following manner. First, the binder resin is mixed with components other than the binder resin as needed. As a result, a mixture is obtained. The resultant mixture is melted and kneaded. The resultant mixture melted and kneaded is crushed by a known scheme to obtain crushed particles. The resultant particles are classified by a known scheme to obtain toner cores **2** having a desired diameter.

Examples of the polymerization method include the following methods. In one example, a mixture melted and kneaded is obtained in the same manner as the melting and kneading method, and the resultant mixture melted and kneaded is sprayed into the air by using a disk or a multi-fluid nozzle to obtain toner cores. In another example, the toner cores are directly generated through suspension polymerization. A yet another example is a dispersion polymerization method for directly generating the toner cores by using an aqueous organic solvent in which a monomer is soluble but a polymer to be obtained is not

soluble. A yet another example is an emulsion polymerization method, such as a so-called soap-free polymerization, of directly generating the toner cores through polymerization caused in the presence of an aqueous polar polymerization initiator. A yet another example is a heteroaggregation method in which polar primary particles are prepared through emulsion polymerization, followed by adding oppositely charged polar particles to cause aggregation.

The following describes different modes of the formation process.

In one mode, the formation process involves an adhering process, a supply process, and a resinifying process (first formation process). In the adhering process, the particulates **4** are caused to adhere to the surfaces of the toner cores **2**. In the supply process, a shell-layer-forming liquid containing a monomer and/or a prepolymer of the thermosetting resin is supplied to the surfaces of the toner cores **2** (first supply process). In the resinifying process, the monomer and/or the prepolymer of the thermosetting resin contained in the shell-layer-forming liquid are resinified (first resinifying process).

When the formation process of forming the shell layers **3** involves the adhering process, the supply process, and the resinifying process, the electrostatic latent image developing toner can be manufactured to have the toner particles **1** containing the inorganic particulates **4** that are evenly dispersed in the shell layers **3**. In addition, the adhering process conducted immediately upon the manufacture of the toner cores **2** can improve the handleability and the fluidity of the toner cores **2** during storage.

In the adhering process, the inorganic particulates **4** are caused to adhere to the surface of each toner core **2** obtained in the preparatory process. The inorganic particulates **4** can be caused to adhere to the surfaces of the toner cores **2** by, for example, mixing the toner cores **2** with the inorganic particulates **4** using a mixer (FM mixer or Nauta mixer (registered trademark)) under the conditions ensuring that the inorganic particulates **4** are not fully embedded in the toner cores **2**.

In the first supply process, the shell-layer-forming liquid is supplied to the surfaces of the toner cores **2**. The shell-layer-forming liquid contains a monomer and/or a prepolymer of the thermosetting resin. Examples of the method for supplying the shell-layer-forming liquid to the toner cores **2** include a method in which the shell-layer-forming liquid is sprayed to the surfaces of the toner cores **2** and a method in which the toner cores **2** are immersed in the shell-layer-forming liquid.

The shell-layer-forming liquid is prepared by, for example, stirring and mixing a solvent, a monomer and/or a prepolymer of the thermosetting resin, and other additives (for example, dispersant, which will be described later) as needed. The solvent is not particularly limited to a specific type, and examples thereof include toluene, acetone, methyl ethyl ketone, tetrahydrofuran, and water.

The monomers of the thermosetting resin described above are appropriately selected. In addition the prepolymers of the thermosetting resin described above are obtained by increasing, the polymerization degree of the monomers of the thermosetting resin to a certain extent to reach the state just before the monomers become polymerized. Therefore, the prepolymers may also be referred to as initial polymers or initial condensate.

The shell-layer-forming liquid may contain a known dispersant to improve the dispersibility of the monomer and/or the prepolymer of the thermosetting resin in a solvent. The content of the dispersant in the shell-layer-forming

liquid is 0.1% by mass or more and 15% by mass or less, for example. With the dispersant content of 0.1% by mass or more in the shell-layer-forming liquid, good dispersibility is ensured. On the other hand, with the dispersant content of 15% by mass or less in the shell-layer-forming liquid, the environmental impact caused by the dispersant can be reduced. The dispersant can be removed by conducting, for example, a washing process after the manufacture of the toner particles **1** or **5** according to the present disclosure.

10 In the first resinifying process conducted after the first supply process, the monomer and/or the prepolymer of the thermosetting resin contained in the shell-layer-forming liquid are resinified into a thermosetting resin through any polymerization or condensation. As a result, the shell layers **3** are formed on the surfaces of the respective toner cores **2**.

15 The scope of the resinification referred herein covers resinification into a resin having a sufficiently high polymerization degree as well as resinification into a resin having a medium polymerization degree.

20 The first resinifying process is carried out at the reaction temperature (resinifying temperature) maintained preferably within the range of 40° C. to 90° C., and more preferably within the range of 50° C. to 80° C. With the reaction temperature of 40° C. or more, the resultant shell layers **3** will have a sufficient hardness. On the other hand, with the reaction temperature of 90° C. or less, the resultant shell layers **3** are prevented from being excessively hard. This ensures that the shell layers **3** can be readily ruptured in response to heat and pressure applied for fixing.

25 In another mode, the formation process involves a second supply process and a second resinifying process (second formation process). In the second supply process, a shell-layer-forming liquid containing a monomer and/or a prepolymer of the thermosetting resin and the inorganic particulates **4** is supplied to the surfaces of the toner cores **2**. In

30 the second resinifying process, the monomer and/or the prepolymer of the thermosetting resin contained in the shell-layer-forming liquid supplied to the surfaces of the toner cores **2** are resinified. When the second formation process is employed for forming the shell layers **3**, each electrostatic latent image developing toner according to the present disclosure can be manufactured through less complicated processes.

35 The method for preparing the shell-layer-forming liquid in the second supply process is not particularly limited. For example, the monomer and/or the prepolymer of the thermosetting resin, the inorganic particulates **4**, and various additives as needed (for example, a positively-charging agent or dispersant) are added to any solvent, appropriately followed by stirring and mixing. The solvent, the monomer and/or the prepolymer of the thermosetting resin, and the dispersant to be used are the same as those used in the preparation of the shell-layer-forming liquid in the first supply process.

40 Examples of the method for supplying the shell-layer-forming liquid to the toner cores **2** in the second supply process include a method in which the shell-layer-forming liquid is sprayed to the surfaces of the toner cores **2** and a method in which the toner cores **2** are immersed in the shell-layer-forming liquid.

45 In the second resinifying process, the monomer and/or the prepolymer of the thermosetting resin are resinified to form the shell layers, and thus the electrostatic latent image developing toner containing the toner particles **1** is obtained. The conditions and scheme for conducting the second resinifying process can be the same as those for conducting the first resinifying process. That is, the second resinifying

process is carried out at the reaction temperature (resinifying temperature) maintained preferably within the range of 40° C. to 90° C., and more preferably within the range of 50° C. to 80° C. With the reaction temperature of 40° C. or more, the resultant shell layers 3 will have a sufficient hardness. On the other hand, with the reaction temperature of 90° C. or less, the resultant shell layers 3 are prevented from being excessively hard and thus can be ruptured easily upon application of heat and pressure for a fixing process.

Up to this point, the manufacturing method according to the present embodiment has been described. The electrostatic latent image developing toner after the formation process of the manufacturing method according to the present embodiment may further be subjected to one or more processes selected from a washing process, a drying process, and an external addition process as needed.

In the washing process, the electrostatic latent image developing toner obtained by conducting the formation process is washed with water, for example.

In the drying process, the electrostatic latent image developing toner having been washed is dried by using, for example, a dryer (such as a spray dryer, a fluidized bed dryer, a vacuum freeze dryer, or a reduced pressure dryer). The use of a spray dryer is preferred for easy suppression of aggregation of the toner particles contained in the electrostatic latent image developing toner being dried. When a spray dryer is used, a dispersion of the external additive 6 (for example, silica particulates) can be sprayed during the drying, for example. Therefore, the external addition process, which will be described later, can be conducted at the same time.

With reference to FIGS. 1 and 3, the following describes the external addition process. In the external addition process, the external additive 6 is caused to adhere to the surface of each toner particle 1. Suitable examples of the method for causing the external additive 6 to adhere include a method in which the electrostatic latent image developing toner containing the toner particles 1 are mixed with the external additive 6 by using a mixer (for example, FM mixer or Nauta mixer (registered trademark)) under the conditions ensuring that the external additive 6 is not embedded in the surfaces of the shell layers 3. As a result, the electrostatic latent image developing toner containing the toner particles 5 is manufactured.

The following describes a method, according to an embodiment of the present disclosure, for fixing an electrostatic latent image developing toner to a recording medium. The fixing method according to the present embodiment involves a toner supplying process and a load applying process. In the toner supplying process, the electrostatic latent image developing toner is supplied to the surface of the recording medium. In the load applying process, a load of 5 N/cm<sup>2</sup> or more and 10 N/cm<sup>2</sup> or less is applied to the recording medium of which the electrostatic latent image developing toner has been supplied to the surface.

In the toner supplying process, a toner image is developed in the following manner before the electrostatic latent image developing toner is supplied to the surface of the recording medium. To develop the toner image by an image forming apparatus, a scheme using, for example, corona discharge is employed to charge the surface of the image bearing member. Thereafter, the charged surface of the image bearing member is exposed to a beam or the like, to electrically neutralize the exposed surface. As a result, an electrostatic latent image is formed on the surface of the image bearing member. Then, the electrostatic latent image developing toner is supplied to the surface of the image bearing member

bearing the electrostatic latent image. The portions of the surface exposed to light attracts the electrostatic latent image developing toner, so that the electrostatic latent image is developed into a toner image. Next, the toner image is transferred from the image bearing member to the recording medium by the transfer roller, so that the electrostatic latent image developing toner is supplied to the recording medium.

In the load applying process, a load of 5 N/cm<sup>2</sup> or more and 10 N/cm<sup>2</sup> or less is applied to the recording medium of which the electrostatic latent image developing toner has been supplied to the surface. As a result, the electrostatic latent image developing toner is fixed to the recording medium.

With reference to FIGS. 1 and 4, the following describes the load applying process in detail. FIG. 4 shows an example of a fixing unit 7 for conducting the load applying process. The fixing unit 7 includes a heating roller 9, a pressure roller 10, a heat source 11, a temperature measuring member 12, and a separating member 13. The heating roller 9 is provided with the heat source 11 (for example, a halogen heater) and heats the recording medium 8 by using the heat source 11. The temperature measuring member 12 controls the temperature of heat applied to the heating roller 9. The pressure roller 10 is disposed to face the heating roller 9 and applies load to the recording medium 8. The separating member 13 separates the recording medium 8 from the heating roller 9 after the load applying process.

More specifically, the fixing unit 7 causes the recording medium 8 to which the electrostatic latent image developing toner has been supplied to pass between the heating roller 9 and the pressure roller 10 so as to apply heat and load to the recording medium 8 and the electrostatic latent image developing toner residing thereon. In response, the shell layers 3 of the toner particles included in the electrostatic latent image developing toner rupture, so that the toner cores 2 melt and soften to be fixed to the recording medium 8. The load applied for fixing can be adjusted by appropriately changing the load applied by the pressure roller 10 the roller and the nip width. The nip width refers to the width across which the pressure roller 10 is in contact with the heating roller 9. Thereafter, the recording medium 8 is peeled away and separated from the heating roller 9 by the separating member 13.

The fixing method according to the present embodiment is a so-called heating and pressurizing method involving the use of a heating roller and a pressure roller. One or more of the inorganic particulates 4 present within the shell layers 3 serve as a starting point of rupturing of the shell layers 3, ensuring that the shell layers 3 readily rupture upon application of heat and pressure. As a result, the fixing temperature and fixing load necessary for fixing the electrostatic latent image developing toner to the recording medium can be substantially reduced.

In the fixing method according to the present embodiment for fixing an electrostatic latent image developing toner, the fixing load can be reduced to fall within the range of 5 N/cm<sup>2</sup> to the 10 N/cm<sup>2</sup>. With the fixing load of 10 N/cm<sup>2</sup> or less, the recording medium is not subjected to an excessive load at the time of the fixing. This improves the durability and conveyance of the recording medium and helps protecting the recording medium from occurrence of defects (such as wrinkles) resulting from the excessive pressure. This additionally helps preventing the deterioration and the cost increase of the component members (especially of the rubber members) of the fixing unit. On the other hand, the fixing load of 5 N/cm<sup>2</sup> or higher improves the fixability.

Note that the fixing load necessary for a typical electrostatic latent image developing toner is 20 N/cm<sup>2</sup> or more and 100 N/cm<sup>2</sup> or less.

With the fixing method according to the present embodiment, the fixing temperature can be reduced as compared with the fixing of an electrostatic latent image developing toner having the shell layers in which no inorganic particulates 4 or spherical or near-spherical inorganic particulates were present within the shell layers. As a result, the load imposed by heat is reduced and thus the durability of the recording medium can be improved. In addition, the deterioration and the cost increase of the component members of the fixing unit can be suppressed.

With the fixing method according to the present embodiment, the fixing time can be 20 msec or more and 70 msec or less, for example. Preferably, the fixing time can be 20 msec or more and 50 msec or less.

### EXAMPLES

The following more specifically describes the present disclosure by way of examples. However, the present disclosure is not limited to these examples.

#### (Preparation of Needle-Like Titanium Oxide Particulates)

##### Titanium Oxide Particulates A

First, metatitanic acid was obtained by a sulfuric acid method. To the metatitanic acid, an aqueous solution of sodium hydroxide (concentration of 50% by mass) was added in an amount equal to 4-fold molar equivalent of titanium oxide, followed by heating at 95° C. for two hours. The resultant was sufficiently washed with pure water. Then, hydrochloric acid (concentration of 31% by mass) was added such that the ratio of hydrogen chloride to titanium oxide (hydrogen chloride/titanium oxide) was equal to 0.26, followed by heating for 1 hour at a temperature keeping the hydrochloric acid boiling. Thereafter, the heated mixture was gradually cooled and neutralized with 1N of the aqueous solution of sodium hydroxide until the pH reached 7. Then, the resultant was washed and dried to prepare rutile-type titanium oxide. To 100 parts by mass of the thus prepared rutile-type titanium oxide, 100 parts by mass of sodium chloride and 25 parts by mass of tetrasodium pyrophosphate decahydrate were added. The resultant was mixed by a vibratory ball mill for one hour to obtain a mixture. The resultant mixture was then baked at 850° C. for 1 hour in an electric furnace to obtain a baked product. The resultant baked product was put into pure water, followed by heating at 80° C. for 6 hours. The resultant was then washed with pure water to remove soluble salt to prepare titanium oxide particulates A. The titanium oxide particulates A have a shape with an aspect ratio of 1.75, an average major diameter of 140 nm, and an average minor diameter of 80 nm.

##### Titanium Oxide Particulates B to I

The titanium oxide particulates B to I having the shapes shown in Table 1 were prepared.

TABLE 1

| Type of titanium oxide particulates | Aspect ratio | Average major diameter nm | Average minor diameter nm |
|-------------------------------------|--------------|---------------------------|---------------------------|
| A                                   | 1.75         | 140                       | 80                        |
| B                                   | 2.00         | 30                        | 15                        |
| C                                   | 2.23         | 290                       | 130                       |
| D                                   | 1.38         | 110                       | 80                        |
| E                                   | 2.38         | 190                       | 80                        |
| F                                   | 1.32         | 290                       | 220                       |

TABLE 1-continued

| Type of titanium oxide particulates | Aspect ratio | Average major diameter nm | Average minor diameter nm |
|-------------------------------------|--------------|---------------------------|---------------------------|
| G                                   | 2.83         | 170                       | 60                        |
| H                                   | 1.08         | 65                        | 60                        |
| I                                   | 2.07         | 310                       | 150                       |

### Example 1

#### Preparatory Process

5 By using an FM mixer, 100 parts by mass of a polyester resin (manufactured by Kao Corporation, an acid value of 16 mgKOH/g, a hydroxyl value of 22 mgKOH/g, a softening point Tm of 100° C., and a glass transition point Tg of 48° C.) was mixed with 5 parts by mass of a colorant (C.I.

10 pigment blue 15:3 type, copper phthalocyanine) and 5 parts by mass of a release agent (ester wax, "WEP-3" manufactured by NOF Corporation) to prepare a mixture. The resultant mixture was melted and kneaded by a two-axis extruder ("PCM-30" manufactured by Ikegai Corp) to obtain 15 kneaded matter. The resultant kneaded matter was pulverized by a mechanical pulverizer ("Turbo Mill" manufactured by FREUND-TURBO CORPORATION), followed by classification by a classifier ("Elbow-Jet" manufactured by 20 Nittetsu Mining Co., Ltd.) to obtain toner cores having a volume median diameter of 6 µm.

#### (Adhering Process)

To the resultant toner cores, the titanium oxide particulates A were added such that the amount of the titanium oxide 25 particulates A adhered was 1% by mass of the total amount of the toner cores. Then, the resultant was mixed by an FM mixer to cause the titanium oxide particulates A to adhere to the surfaces of the toner cores.

#### (Supply Process)

30 A 1-liter, three-necked flask was set in a water bath kept at 30° C. In the flask, the pH of the ion exchanged water (300 mL) was adjusted to 4 by using hydrochloric acid. In the resultant ion exchanged water, 2 mL of an aqueous solution containing initial polymers of methylol melamine ("Mirben resin SM-607" manufactured by Showa Denko K.K., a solid concentration of 80% by mass) was dissolved to obtain a shell-layer-forming liquid. To the shell-layer-forming liquid, 300 g of the toner cores resulting from the adhering process were added.

#### (Resinifying Process)

35 The shell-layer-forming liquid and the toner cores were stirred at 200 rpm for one hour. Then, 500 mL of the ion exchanged water was added to the flask. While the content of the flask was stirred at 100 rpm, the temperature inside the 40 flask was raised up to 70° C. at the heating rate of 1° C./min. After the temperature rise, the content of the flask was kept stirring for 2 hours at 70° C. at 100 rpm. Subsequently, sodium hydroxide was added to adjust the pH of the flask content to 7. Then, the content of the flask was cooled to 45 room temperature to obtain a liquid containing the electrostatic latent image developing toner.

#### (Washing Process)

50 From the liquid containing the electrostatic latent image developing toner, wet cake of the toner was filtrated out by 55 using a Büchner funnel. The wet cake of the toner was again dispersed in ion exchanged water to wash the toner. The process of filtrating and dispersing were repeated five times.

## (Drying Process)

First, 2 g of the collected electrostatic latent image developing toner was dispersed in 20 g of water to obtain a dispersion. The toner was collected when the conductivity of the dispersion reached 10  $\mu$ S/cm. Then, the collected toner was dried by being left to stand for 48 hours in an atmosphere of 40° C.

## (External Addition Process)

To the surfaces of the toner particles in the toner thus dried, dry silica (particle diameter: 0.1  $\mu$ m) was added as an external additive such that the amount of the dry silica added was 0.5% by mass with respect to the total amount of the toner. As a result, the electrostatic latent image developing toner of Example 1 was obtained. This electrostatic latent image developing toner was subjected to the evaluation, which will be described later. Table 2 shows the evaluation results of the electrostatic latent image developing toner of Example 1. In addition, FIG. 5 shows an SEM photograph ( $\times 30,000$  magnification) of the electrostatic latent image developing toner. As is clear from FIG. 5, in the electrostatic latent image developing toner of Example 1, the dried silica was uniformly adhered to the surfaces of the toner particles. FIG. 6 shows an SEM photograph ( $\times 30,000$  magnification) of the electrostatic latent image developing toner after the fixing process. As is clear from FIG. 6, in the electrostatic latent image developing toner of Example 1, the shell layers were ruptured by the titanium oxide particulates through the fixing process, and the toner cores was melted to flow out in a narrow stream through the ruptured portion of the shell layers.

## Example 2

The electrostatic latent image developing toner of Example 2 was obtained in the same manner as Example 1, except that the titanium oxide particulates A were changed to the titanium oxide particulates B.

## Example 3

The electrostatic latent image developing toner of Example 3 was obtained in the same manner as Example 1, except that the titanium oxide particulates A were changed to the titanium oxide particulates C.

## Example 4

The electrostatic latent image developing toner of Example 4 was obtained in the same manner as Example 1, except that the titanium oxide particulates A were changed to the titanium oxide particulates D.

## Example 5

The electrostatic latent image developing toner of Example 5 was obtained in the same manner as Example 1, except that the titanium oxide particulates A were changed to the titanium oxide particulates E.

## Example 6

The electrostatic latent image developing toner of Example 6 was obtained in the same manner as Example 1, except that the titanium oxide particulates A were changed to the titanium oxide particulates F.

## Comparative Example 1

The electrostatic latent image developing toner of Comparative Example 1 was obtained in the same manner as

Example 1, except that the titanium oxide particulates A were changed to the titanium oxide particulates G.

## Comparative Example 2

The electrostatic latent image developing toner of Comparative Example 2 was obtained in the same manner as Example 1, except that the titanium oxide particulates A were changed to the titanium oxide particulates H.

## Comparative Example 3

The electrostatic latent image developing toner of Comparative Example 3 was obtained in the same manner as Example 1, except that the titanium oxide particulates A were changed to the titanium oxide particulates I.

## Comparative Example 4

The electrostatic latent image developing toner of Comparative Example 4 was obtained in the same manner as Example 1, except that no titanium oxide particulates were contained.

Table 2 shows the evaluation results of the respective electrostatic latent image developing toners obtained in Examples 2 to 6 and Comparative Examples 1 to 4.

The following describes the evaluation method and the measurement method used for the respective electrostatic latent image developing toners obtained in Examples and Comparative Examples.

## (1) Evaluation of Ghost Occurred in Developing Process

To evaluate each of Examples and Comparative Examples, 10 parts by mass of a corresponding toner was mixed with 90 parts by mass of a carrier (carrier for FS-05300DN) for 30 minutes by a ball mill to prepare a two-component developer. As the evaluation equipment, a printer ("FS-05250DN" manufactured by KYOCERA Document Solutions Inc.) was altered to have a function of adjusting the fixing temperature. Each two-component developer prepared as above was put into a toner container of the developing device of the evaluation equipment. After the evaluation equipment was powered on and ready for stable operation, an image was printed and this image was determined as the initial image. Subsequently, 100,000 prints of an image with the coverage rate of 4% or more and 5% or less were continuously produced in a normal temperature and humidity environment (temperature range: 20° C. or more and 23° C. or less, relative humidity: 50% RH or more and 65% RH or less). Thereafter, a solid image was printed.

The initial image and the solid image (the image after the 100,000 prints continuously produced) were measured for their image densities (ID), brightness ( $L^*$ ), hue ( $a^*$ ), and hue ( $b^*$ ) by using a Macbeth reflection densitometer ("SPM-50" manufactured by SAKATA INX ENG. CO., LTD). Then, the value of  $\Delta E$  was calculated by using the following formula, and the evaluation was made in accordance with the following criteria.

$$\Delta E = \sqrt{(a^*)^2 + (b^*)^2 + (L^*)^2}$$

Very Good: The value of  $\Delta E$  is 3 or less.

Good: The value of  $\Delta E$  is more than 3 and less than 5.

Poor: The value of  $\Delta E$  is 5 or more.

## (2) Evaluation of Image Deterioration

In the same manner as described above regarding "(1) Evaluation", an initial image as well as a solid image after 100,000 prints continuously produced were obtained. The

initial image and the solid image were measured for their image densities (ID) and fogging values (FD) by using a Macbeth reflection densitometer ("SPM-50" manufactured by SAKATA INX ENG. CO., LTD). In addition, the initial image and the solid image were visually inspected. The evaluations were made in accordance with the following criteria.

Very Good: The value of ID is 1.30 or more, FD is less than 0.005, and no inconsistencies in the image.

tube. The heating roller is provided with a halogen heater disposed inside the heating roller and is heated by radiation heat of the heater. The heating roller is provided with a temperature measuring member to measure the temperature of the heating roller, and the power supply to the heater is controlled based on the measurement results. The pressure roller includes a core bar ( $\phi 12$  mm), an 8-mm-thick silicone rubber layer coating the core bare, and a paraformaldehyde resin tube coating the silicone rubber layer.

TABLE 2

| Aspect ratio          | Average major diameter (nm) | Average minor diameter (nm) | Development ghost | Initial           |           |     | Image inconsistencies | Image deterioration | After 100,000 prints |    |           |            |       |
|-----------------------|-----------------------------|-----------------------------|-------------------|-------------------|-----------|-----|-----------------------|---------------------|----------------------|----|-----------|------------|-------|
|                       |                             |                             |                   | Development ghost |           | ID  |                       |                     | Development ghost    |    | ID        | FD         |       |
|                       |                             |                             |                   | 4E                | ID        | 4E  |                       |                     | ID                   | 4E | ID        | Fixability |       |
| Example 1             | 1.75                        | 140                         | 80                | 2                 | Very good | 1.4 | 0.001                 | No                  | Very good            | 4  | Good      | 1.3        | 0.003 |
| Example 2             | 2.00                        | 30                          | 15                | 2                 | Very good | 1.4 | 0.002                 | No                  | Very good            | 3  | Very good | 1.3        | 0.003 |
| Example 3             | 2.23                        | 290                         | 130               | 2                 | Very good | 1.4 | 0.002                 | No                  | Very good            | 3  | Very good | 1.2        | 0.001 |
| Example 4             | 1.38                        | 110                         | 80                | 2                 | Very good | 1.4 | 0.001                 | No                  | Very good            | 4  | Good      | 1.3        | 0.003 |
| Example 5             | 2.38                        | 190                         | 80                | 2                 | Very good | 1.4 | 0.001                 | No                  | Very good            | 3  | Very good | 1.2        | 0.001 |
| Example 6             | 1.32                        | 290                         | 220               | 2                 | Very good | 1.4 | 0.001                 | No                  | Very good            | 4  | Good      | 1.2        | 0.001 |
| Comparative Example 1 | 2.83                        | 170                         | 60                | 2                 | Very good | 1.4 | 0.001                 | No                  | Very good            | 5  | Poor      | 1.0        | 0.015 |
| Comparative Example 2 | 1.08                        | 65                          | 60                | 2                 | Very good | 1.4 | 0.002                 | No                  | Very good            | 5  | Poor      | 1.0        | 0.015 |
| Comparative Example 3 | 2.07                        | 310                         | 150               | 2                 | Very good | 1.4 | 0.002                 | No                  | Very good            | 6  | Poor      | 0.9        | 0.017 |
| Comparative Example 4 | No titanium oxide           |                             |                   | 2                 | Very good | 1.4 | 0.002                 | No                  | Very good            | 6  | Poor      | 0.9        | 0.017 |

Good: The value of ID is 1.10 or more and less than 1.30, FD is 0.005 or more and less than 0.015, and no inconsistencies in the image.

Poor: The value of ID is less than 1.10, FD is 0.015 or more, and inconsistencies observed in the image.

### (3) Fixing Temperature (Low-Temperature Fixability)

Each of the electrostatic latent image developing toners of Examples and Comparative Examples was subjected to the fixing process with the use of a heating and pressurizing fixing unit as shown in FIG. 4. Then, the temperature at the time of each fixing process was measured. More specifically, the fixing temperature was changed from 100°C. to 200°C. in steps of 5°C. and the fixing state of 1.0 mg/cm<sup>2</sup> electrostatic latent image developing toner on 90 g/m<sup>2</sup> paper was visually inspected. The lowest temperature at which the toner was favorably fixed was determined as a lowest fixing temperature. Note that the lowest temperature was measured under the conditions of the fixing speed of 230 mm/sec, the nip width of 8 mm, and the nip passage time of 35 msec. The evaluations were made in accordance with the following criteria.

Very Good: The fixing temperature is 150°C. or less.

Good: The fixing temperature is 155°C.

Poor: The fixing temperature is 160°C. or more.

The following describes the structure of the fixing unit used in the measurements and evaluations. The heating roller includes a core bar ( $\phi 26$  mm) made of 1-mm-thick aluminum and a 300-nm-thick silicone rubber layer coating the core bar. The silicone rubber layer is coated with a release layer that is a 30-nm-thick paraformaldehyde resin

In each electrostatic latent image developing toner according to Examples of the present disclosure, the inorganic particulates were present within the shell layers. As is apparent from Table 2, each electrostatic latent image developing toner according to Examples of the present disclosure maintained appropriate chargeability for a long time. Consequently, even after 100,000 prints were continuously produced, occurrence of image ghost and image deterioration was suppressed, and high image quality was ensured. In addition, the inorganic particulates served as a starting point of the shell layer rupturing, the low-temperature fixability was significantly improved.

In the electrostatic latent image developing toner of Comparative Example 1, the inorganic particulates having an aspect ratio exceeding 2.5 were present within the shell layers. Therefore, the chargeability of the toner significantly decreased to promote the charge leakage more than necessary. As a result, after 100,000 prints were continuously produced, the toner amount on the development sleeve increased and thus that the residual toner on the development sleeve was not sufficiently collected. This led to occurrence of ghost in the developing process. In addition, the chargeability of the toner excessively decreased, which led to image deterioration.

In the electrostatic latent image developing toner of Comparative Example 2, the inorganic particulates having an aspect ratio less than 1.25 were present within the shell layers. That is, the shape of the inorganic particulates was more spherical, which is assumed to have caused the decrease in the charge leakage and thus a large amount of charges accumulated on the toner. As a result, the amount of

## 23

charges on the toner increased to the level of overcharging. Thus, after 100,000 prints was continuously produced, the electrostatic adsorption of the toner to the development sleeve increased, which led to a failure of sufficiently collecting the toner and to occurrence of ghost in the developing process. In addition, since the shape of inorganic particulates was more spherical, the concentration of the stress applied to the inorganic particulates was reduced. This led to a failure in providing a starting point for the shell layer rupturing. Therefore, the low-temperature fixability of the toner did not improve. 10

In the electrostatic latent image developing toner of Comparative Example 3, the shell layers contained therein inorganic particulates having an average major diameter exceeding 300 nm. As a result, the inorganic particulates were detached from the surfaces of the toner particles, resulted in that the components of the toner cores, such as wax, were exposed on the surfaces. Thus, as a result of 100,000 prints continuously produced, the adsorption of the toner to the development roller was increased, leading to the toner to adhere to the development sleeve or to occurrence of ghost in the developing process. In addition, as the inorganic particulates were detached or broken, less starting points were provided for shell layer rupturing. Therefore, the low-temperature fixability of the toner did not improve. 15

In the electrostatic latent image developing toner of Comparative Example 4, no inorganic particulates were present within the shell layers. It is therefore assumed that the toner did not exhibit the charge leakage, which resulted in that a large amount of charges accumulated on the toner. As a result, the amount of charges on the toner increased to the level of overcharging. Thus, after 100,000 prints were continuously produced, the electrostatic adsorption of the toner to the development sleeve increased, this led to a failure of sufficiently collecting the toner and to occurrence of ghost in the developing process. In addition, no starting point for the shell layer rupturing was provided, the low-temperature fixability of the toner did not improve. 20

What is claimed is:

1. A method for manufacturing an electrostatic latent image developing toner, comprising: 40  
preparing toner cores containing a binder resin; causing needle-like inorganic particulates to adhere to the respective toner cores; and forming shell layers to coat surfaces of the respective toner cores and the inorganic particulates, wherein the shell layers contain a thermosetting resin, and the needle-like inorganic particulates are present between the toner cores and the shell layers, the inorganic particulates having an aspect ratio of 1.25 or more and 2.5 or less, and 45

## 24

an average major diameter and an average minor diameter of 15 nm or more and 300 nm or less. 5

2. A method for manufacturing an electrostatic latent image developing toner, according to claim 1, wherein the forming of the shell layers involves

supplying a shell-layer-forming liquid to the surface of each toner core to which the needle-like inorganic particulates adhere, the shell-layer-forming liquid containing a monomer and/or a prepolymer of the thermosetting resin, and resinifying the monomer and/or the prepolymer of the thermosetting resin. 15

3. A method for manufacturing an electrostatic latent image developing toner, according to claim 1, in the forming shell layers, the thermosetting resin contains a melamine resin or a urea resin. 20

4. A method for manufacturing an electrostatic latent image developing toner, according to claim 1, in the causing needle-like inorganic particulates to adhere to the respective toner cores, the toner cores are mixed with the inorganic particulates using a mixer. 25

5. A method for manufacturing an electrostatic latent image developing toner, according to claim 2,

in the resinifying, the thermosetting resin is obtained through polymerization or condensation of the monomer and/or the prepolymer of the thermosetting resin. 30

6. A method for manufacturing an electrostatic latent image developing toner, according to claim 1,

in the causing needle-like inorganic particulates to adhere to the respective toner cores, the inorganic particulates are not embedded in the toner cores. 35

7. A method for manufacturing an electrostatic latent image developing toner, according to claim 2,

in the supplying a shell-layer-forming liquid, the shell-layer-forming liquid contains an aqueous medium. 40

8. A method for manufacturing an electrostatic latent image developing toner, according to claim 7,

in the supplying a shell-layer-forming liquid, the aqueous medium is adjusted to pH 4. 45

9. A method for manufacturing an electrostatic latent image developing toner, according to claim 8,

in the supplying a shell-layer-forming liquid, the monomer and/or the prepolymer of the thermosetting resin is added to the aqueous medium. 50

10. A method for manufacturing an electrostatic latent image developing toner, according to claim 2,

in the supplying a shell-layer-forming liquid, the toner cores adhering to the inorganic particulates are added to the shell-layer-forming liquid.

\* \* \* \* \*